

April 8, 1941.

J. H. KNAPP

2,237,785

## METHOD FOR HEAT TREATING IN A SEMIMUFFLE TYPE FURNACE

Filed Feb. 27, 1939



JAMES H. KNAPP,  
INVENTOR.

By *John*

ATTORNEY

## UNITED STATES PATENT OFFICE

2,237,785

## METHOD FOR HEAT TREATING IN A SEMI-MUFFLE TYPE FURNACE

James H. Knapp, Beverly Hills, Calif., assignor to  
 James H. Knapp Co., Los Angeles, Calif., a corporation of California

Application February 27, 1939, Serial No. 258,639

1 Claim. (Cl. 148—16)

My invention relates to the art of heat treating metal and relates more particularly to a method whereby the metal being heat treated is surrounded with a suitable gaseous atmosphere which will not oxidize or decarburize the metal. It was heretofore common practice in the art to heat treat by use of furnaces heated by solid fuel, such as coal and coke, and later by furnaces using fuel gas or oil, the furnaces being so constructed that the work was enveloped by the products of combustion of the burning fuel. These gases of combustion had a harmful effect on the work and caused the surfaces to oxidize, carburize, or decarburize.

Numerous inventors sought to eliminate the disadvantages of such prior art furnaces and methods, such, for example, as by a muffle type furnace in which the treating chamber was separated from the combustion chamber to prevent the products of combustion from enveloping the work and in which separate means was provided for maintaining a suitable atmosphere in the heat treating chamber which would not cause the work to scale. The disadvantages were also overcome by Hayes in Patent No. 1,808,721, issued June 2, 1931, by providing an electrically heated furnace, the electrical heating means, of course, producing no products of combustion, and by providing a gaseous enveloping atmosphere in the treating chamber by introducing an especially proportioned atmosphere of products of combustion which would prevent the formation of scale on the work.

It is an object of my invention to provide a direct fired or semi-muffle furnace in which the products of combustion of the fuel gas envelop the work being treated, and in which there are means for introducing into the combustion chamber substances which will be chemically converted into suitable gases which will mix with the gases of combustion and form a substantially neutral gaseous atmosphere which will not cause the work to scale.

It is another object of my invention to provide a method of heat treating in which the products of combustion of the fuel burned to heat the work are caused to envelop the work and which contain the necessary constituents in proper amounts to prevent scale from forming on the work.

It is another object of my invention to provide a method of heat treating in which the fuel gas and oxygen bearing gas are combusted to produce heat for heating the work to be heat treated, and in which the combustion takes place in the presence of a hydrocarbon gas and/or ammonia or other hydrogen producing gas to produce a resultant mixture of gases which forms a gaseous envelope which is caused to envelop the work for heating the same and for preventing scale.

Other objects of my invention will be brought

out during the course of the following description of a preferred embodiment of my method and apparatus. It should be understood that various changes in substances and proportions and precise steps may be made within the principle of my invention and without departing from the spirit and scope thereof as defined in the appended claims.

In the drawing:

Fig. 1 is a vertical sectional view of a furnace incorporating the features of my invention, this view being taken as indicated by the arrows 1—1 of Fig. 2.

Fig. 2 is a section taken as indicated by the arrows 2—2 of Fig. 1.

Referring to the drawing in detail, there is a suitable frame structure 11 which supports the furnace. The furnace has a floor 12, side walls 14, a rear wall 15, a front wall 16, and a roof 17. The front wall 16 is provided with a doorway or entrance 19 which may be closed by a door 20. Supported within the furnace is a hearth 21 which is supported on suitable supporting blocks 22. This provides the interior of the furnace with a treating chamber 24, a combustion chamber 25, and passages 26 which connect the heating and combustion chambers 24 and 25.

Extended inwardly into openings 27 formed in the side walls 14 are burners 28 which are connected by pipes 29 to a manifold 30, in the form of the invention illustrated there being two burners 28 on each side of the furnace. Connected to the manifold 30, as illustrated in Fig. 2, is a supply line 31 which is connected to a blower 32 which supplies air or other oxygen bearing gas in amounts determined by the position of the air valve 33. For the purpose of supplying fuel gas to the line 31, there is provided in this line 31 a Venturi means 34 to which a fuel gas pipe 35 having a fuel gas valve 36 is connected. For the purpose of supplying a hydrocarbon gas or other carbon monoxide forming gas and for supplying ammonia or other hydrogen forming gas, I provide a Venturi means 38 to which a pipe 39 is connected, this pipe 39 having a hydrocarbon gas branch 40 and an ammonia branch 41, these branches having valves 42 and 43, respectively.

The method of my invention is performed as follows: The blower 22 is placed in operation and the valves 33 and 36 are opened in amounts to supply a predetermined mixture of combustible and oxygen bearing gases in amounts which will produce the desired temperature in the heat treating chamber 24. This combustible mixture is conveyed through the line 31 to the manifold 30 and thereafter passes through the burners 28 into the chamber 25 where it is ignited and combustion takes place so as to produce heat and gases or products of combustion. These products of combustion pass upwardly through the

passages 26 into the heat treating chamber 24 and thus envelop the work being heat treated.

In the combusting of ordinary fuel gases the products of combustion may contain CO<sub>2</sub>, CO, H<sub>2</sub>O, O<sub>2</sub>, CH<sub>4</sub>, N<sub>2</sub>, and H<sub>2</sub>, depending upon the nature of the fuel and the fuel air ratio employed. Under certain conditions the O<sub>2</sub>, CO<sub>2</sub>, and H<sub>2</sub>O would produce scaling or oxidization of the work being heat treated, CO and CH<sub>4</sub> would produce carburization, and O<sub>2</sub>, CO<sub>2</sub>, and H<sub>2</sub> would produce decarburization, while CO and H<sub>2</sub> would produce a reduction of oxides. It will be understood that the gases present and the proportions of gases present in the products of combustion depend upon the fuel gas which is used and upon the fuel gas-air ratio. Where there is a high fuel gas to air ratio, products of combustion ordinarily contain CO<sub>2</sub>, CO, H<sub>2</sub>O, CH<sub>4</sub>, N<sub>2</sub>, and only a slight trace of O<sub>2</sub>, whereas with a lower fuel gas to air ratio there is ordinarily present greater proportions of CO<sub>2</sub> and O<sub>2</sub> with H<sub>2</sub>O and N<sub>2</sub> and possibly no CO or CH<sub>4</sub>. It is generally considered preferable to set the fuel gas to air ratio at a proportion to obtain the highest possible CO<sub>2</sub> and to have present a small percentage of CO but with the lowest practical percentage of O<sub>2</sub>.

In the practice of my process I add the necessary constituents to the gases of combustion to obtain a balanced or neutral condition so that the decarburizing effect of some of the gases will be offset by the carburizing effect of others and the oxidizing effect of some of the gases will be offset by the reducing effect of others. In the process the valve 42 is opened to supply a hydrocarbon gas, such as propane, and the valve 43 is opened to supply a hydrogen forming gas, such as ammonia. The hydrocarbon gas under the action of heat in the combustion chamber breaks down and supplies the necessary carbon to form carbon monoxide and some hydrogen, and the ammonia breaks down and supplies hydrogen and nitrogen. To increase the carbon monoxide content of the enveloping gaseous atmosphere which is introduced into the treating chamber, more hydrocarbon gas is used, and to increase the hydrogen content, more ammonia is used. It will be understood that the main function of the propane or hydrocarbon gas is to furnish carbon for the production of carbon monoxide and that other hydrocarbon gases, such as butane, methane, ethane, etc., may be employed or, in lieu thereof, carbon may be furnished by a partial burning of solid carbon, such as charcoal. In place of ammonia other gases which will produce hydrogen may be employed or, if desired, hydrogen gas may be introduced.

I prefer to introduce these gases to the combustible mixture so that a thorough mixture will be had when the gases pass through the manifold 30 and burners 28. This may be conveniently done, since the volume of the gases which are added are very slight in comparison with the volume of fuel gas and air. If desired, however, these added gases may be introduced directly into the combustion chamber where they will be subjected to the action of the heat without pre-mixing with the combustible gases and will be converted into carbon monoxide and hydrogen, depending upon the amounts of gases so introduced.

It has been found that the percentages of CO and H<sub>2</sub> furnish a satisfactory index for the

nature of the gaseous atmosphere in the heat treating chamber and satisfactory results may be obtained at various temperatures with percentages of these gases ranging from 4% to 30% by volume. In actual practice in a small semi-muffle tool furnace of the type shown in the drawing best results have been obtained over a temperature range of from 1400° F. to 2300° F. with approximately 5% by volume of CO and 25% by volume of H<sub>2</sub>, while with percentages of approximately 10% CO and 10% H<sub>2</sub> or other variations of the above percentages good results have been obtained, but in the experiments conducted the results with these latter mentioned percentages were found to be limited to lower temperature ranges. The amounts of hydrocarbon gas and ammonia or its equivalent introduced may be readily varied by adjusting the valves 42 and 43, and these proportions may be varied in order to obtain the desired percentages of carbon monoxide and hydrogen so as to obtain a balanced or neutral gaseous atmosphere in the heat treating chamber.

I have found that for the lower temperature ranges in the heat treating chamber 24 of between 1400° F. and 1600° F. with certain fuel gases the fuel gas to air ratio can be set high enough in fuel gas so as to produce sufficient CO in the gaseous atmosphere, and that it is only necessary to add ammonia or other hydrogen producing gas to obtain the necessary hydrogen percentage. However, in higher temperatures of from 1600° F. to 2300° F., such a fuel gas-air ratio can not produce the necessary combustion temperature and therefore can not be economically used for these higher temperature ranges, and that, therefore, for these higher temperature ranges it is necessary to add the hydrocarbon gas. It should be understood, however, that my invention is applicable for use where any of the heat treating temperatures are employed and more satisfactory results, both from the type of gaseous atmosphere which is produced and from the standpoint of economy, can be obtained where the hydrogen gas and/or ammonia are added in accordance with the teachings of my process.

In the foregoing description I have disclosed the apparatus of my invention and the preferred process of my invention and have indicated the various elements and percentages which have been found satisfactory. It should be understood, however, that my invention is not limited to the details disclosed herein but extends to all apparatus and all processes incorporating the principle thereof and which fall within the spirit and scope of the appended claim.

I claim as my invention:

In a method of heat treating which includes the steps of: mixing with predetermined proportions of a combustible mixture of combustible and oxygen bearing gases hydrocarbon gas and hydrogen producing gas; combusting the combustible mixture to produce heat and products of combustion and to convert by the action of heat the hydrocarbon gas and hydrogen producing gas into carbon monoxide and hydrogen and thereby form a substantially non-scaling atmosphere; and enveloping the work to be heat treated with said gaseous atmosphere to heat and prevent scaling of the work.